# EUROPEAN PATENT SPECIFICATION

(11) **EP 3 209 806 B1**
(45) Date of publication and mention of the grant of the patent: **25.11.2020**
(21) Application number: 15808458.2
(22) Date of filing: 21.10.2015
(51) Int. Cl.: C21D 8/00, C22C 38/00

(54) **AN ULTRA-HIGH STRENGTH THERMO-MECHANICALLY PROCESSED STEEL**
ULTRAHOCHFESTER THERMOMECHANISCH BEHANDELTER STAHL
ACIER TRAITÉ THERMOMÉCANIQUEMENT À TRÈS HAUTE RÉSISTANCE

(30) Priority: 21.10.2014 IN 3355MU2014
(43) Date of publication of application: 30.08.2017
(73) Proprietor: Bharat Forge Limited, Pune 411036 (IN); Saarloha Advanced Materials Private Limited, Pune, 411036 MAH (IN)
(72) Inventor: KALYANI, Babasaheb Neelkanth, Pune 411036 (IN); TAKALE, Madan Umakant, Pune 411036 (IN); DR. GNANA, Prakasam Balachandran, Pune 411036 (IN); DR. SINGH, Rajkumar Prasad, Pune 411036 (IN); CHAUTHAI, Abhay Ramchandra, Pune 411036 (IN); ARANGI, Suresh Babu, Pune 411036 (IN); MANE, Rajesh Surendra, Pune 411036 (IN); DHARMESH, Kumar, Pune 411036 (IN); PERLA, Srinivas, Pune 411036 (IN); PAWAR, Vinayak Pralhad, Pune 411036 (IN); JADHAV, Shital Shahaji, Pune 411036 (IN)
(74) Representative: Boult Wade Tennant LLP
(86) International application number: PCT/IB2015/058107
(87) International publication number: WO 2016/063224

(56) References cited:
- CN-A- 101 613 830
- JP-A- H09 241 750
- JP-A- 2011 168 820
- JP-A- 2012 158 827
- US-A- 5 762 725
- US-A1- 2004 149 359

## Description

### Field of the Invention:

The present invention relates to ultra-high strength steel for structural components. In particular, it relates to the process of making such steel that has a desirable microstructure in the thermo-mechanically processed and differently cooled conditions that delivers high fatigue resistance in service. The steel and the process of its manufacturing technique enables manufacture of components that exhibit bainitic microstructure that impart ultra-high strength ranges with very high fatigue resistance properties.

The steel and its method of manufacturing process enables saving in alloying additives compared to hardened and tempered alloy steels and in addition avoid expensive heat treatment operations to achieve the desired range of mechanical properties. The steel developed in the present invention is a suitable replacement for microalloyed steel bars used for structural component development. The steel can be used for applied as the hot rolled and air cooled long products that can be directly used for applications or it can be directly hot forged in open or closed die forging followed by controlled cooling to achieve the desired microstructure and range of mechanical properties. The ultra-high strength steel (UTS in the 1100 to 1420 MPa range) of the invention provides a competitive replacement for quench tempered alloy steels in terms of strength and fatigue, ductility, although its toughness is lower compared to Quenched and Tempered steels but superior to micro alloyed steels. Thus, the potential steel bar product can be applied in various industries that include automotive, railways, general engineering, agricultural implements, construction, mining shafts, etc. The steel exhibits unique range of mechanical properties that develops due to the process of invention which involves the steel chemistry and the thermo-mechanical processing followed by controlled cooling.

### Background of the invention:

High performance and weight reduction of dynamic components in engineering machines is a major driver for achieving fuel efficiency. In automotive industry, even small weight reduction in dynamic engine components translates into significant fuel efficiency and overall weight savings in the structure. Products such as bars, tubes/pipes, and other solid products such as axles, typically termed as 'long' products, made of steel and produced using minor addition of additives such as Vanadium (V), Niobium (Nb) and Titanium (Ti) and with ferrite pearlite microstructures have long dominated the markets. These materials, which have been competing with alloy steel in terms of achieving the required strength, are produced using thermo-mechanical processes with controlled cooling, which completely avoid subsequent quenching and tempering heat treatment of the component. The micro alloyed steels are known to have ultimate tensile strength (UTS) upto1000 MPa although they have lower impact toughness.

CN101613830A discloses a hot rolled bainitic steel rail and a production process.

US2004/149359A1 discloses a method of fabricating a steel forging, and a forging obtained thereby.

The present invention relates to innovative composition of a steel and associated thermo-mechanical processing of making it, such that it has desirable microstructure that gives ultra-high strength and fatigue resistance. The mechanical properties of the invented steel shows values of ultimate tensile strength (UTS) between 1100 and 1420 MPa; yield stress (YS) between 700 and 1030 MPa; percentage elongation (% E) =10 to 18%; % reduction in area between 32 and 50 %, Charpy V-notch Impact toughness greater than 20 J/cm² and hardness greater than 330HBW. Higher strengths were obtained with increasing cooling rate after thermo-mechanical processing. The fatigue properties of the steel rolled bar of the invention have been found to exhibit greater than 5 million cycles with rotating bending type testing at a stress level of 515MPa. It was also found that the fatigue life of the forged component of the invention is at least five times more than that of the existing alloy steel materials.

### Summary of the Invention:

The present invention describes the steel composition and the entire process of making the steel from melting to thermo-mechanical processing to achieve steel with ultra-high strength and very high fatigue performance. Specifically, the invention relates to an ultra-high strength steel in accordance with claim 1, a process of making an ultra-high strength steel rolled bar in accordance with claim 2, and a process of making forged components in accordance with claim 3.

### Objects of the Invention:

The object of the present Invention is to develop an ultra-high strength steel with high fatigue resistance with thermo-mechanically processed and control cooled steel that is processed with induction or electric arc furnace or Basic oxygen furnace routes followed by secondary refining, vacuum degassing and traditional casting processes such as ingot casting or continuous casting.

Another object of the present investigation is to achieve a wide range of mechanical properties within Ultra high strength range by changing the cooling rate post thermo-mechanical processing in air, water, polymer, oil and vermiculite cooling.

Another object of the present invention is to propose usefulness of steel in weight reduction by at least 10% as a substitute for heat treated alloy steels or microalloyed steels.

Another object of the invention is to minimize the cost of steel manufacturing as compared to alloy steels and savings associated with avoidance of heat treatment in alloy steels.

Another object of present invention is to produce ultra-high strength components having fatigue resistance of at least five times compared to regular heat treated or micro alloyed steels.

### Brief Description of Figures:

Figure 1 Manufacturing method process flow of ultra-high strength steel.
Figure 2 Microstructure of the steel made at various cooling conditions showing the bainitic microstructure obtained at various processing conditions
Figure 3: Automotive front axle beam manufactured using ultra-high strength steel grade.
Figure 4 Microstructure of the forging with invented ultra-high strength steel.

### Detailed Description of the Invention

The present invention describes the development of ultra-high strength steel for potential use in light weighting and fatigue resistant component applications.

The primary steel is manufactured using induction furnaces, electric arc furnaces (EAF), ladle furnaces or basic oxygen furnaces. The primary steel is suitably alloyed in a secondary refining furnace followed by vacuum degassing to produce the steel of designed chemistry additives shown in Table 1, based on theoretical considerations on alloy design principles. The steel is refined and killed with Aluminium (Al) to get a residual oxygen level to less than 15ppm. This is found to reduce the potential oxide inclusions that have an effect on the fatigue life of the component that may be made using the steel of the present invention.

**Table 1: Composition of the steel designed for meeting Ultra high strength range and fatigue resistance. [Composition in % w/w]**

| **Elements** | **C** | **Mn** | **Si** | **S** | **P** | **Cr** | **Ni** | **Mo** | **V** | **Al** | **B** | **Ti** | **Nb** | **O** |
|---|---|---|---|---|---|---|---|---|---|---|---|---|---|---|
| Min | 0.10 | 1.2 | 0.5 | | | 0.8 | 0 | 0.05 | - | - | | 0.010 | 0.05 | |
| Max | 0.25 | 2.5 | 1.7 | 0.03 | 0.02 | 1.4 | 0.4 | 0.1 | 0.1 | 0.02 | 0.003 | 0.035 | 0.10 | 0.0015 |

The steel is cast through ingot casting preferably with bottom pouring up-hill casting technique or it may be cast as a concast steel product of suitable size. The as-cast ingot or the concast bloom may be hot charged or cold charged in a furnace for further deformation. The initial soaking for hot deformation is done at a temperature between 1280° C and 1220° C. The soaked bloom is subject to hot rolling. Suitable reduction per pass is applied. The material gets deformed easily by forging or directly hot rolling with good surface finish. The hot worked material is suitably hot finished at a temperature between 1000 and 900° C. This is followed by control cooling the deformed steel in any of the cooling medium vermiculite, air, oil, polymer or water. The distortion of the steel is depending on the quenching severity of the media. The steel quenched in water or polymer may require a stress relief temper treatment at a temperature between 200 and 340 °C.

The invention discloses development of the steel and its processing where the content, morphology and distribution of the phases ensure the unique range of mechanical properties. The bainitic transformation involves a displacive transformation followed by diffusion of carbon to form carbides that create the bainitic microstructures.

The invention discloses the stability of predominantly bainitic microstructure when control cooled in various media such as vermiculite, air, oil, polymer and water quenching which resulted in higher strength.

The invention also discloses development of steel which can be made at par with that of processing an air cooled micro alloyed steel but delivers ultra-high strength level and superior fatigue resistance.

In one typical embodiment, the primary steel was melted in a 35MT electric arc furnace followed by secondary steel making using a ladle furnace. The entire process flow followed is shown in Figure 1. The process of the present invention ensures that the steel developed by adopting above mentioned process has Oxygen content less than 15ppm (a condition that is necessary to give ultra-high strength). Secondary steel making followed by vacuum degassing ensures low gas content. One advantage of completely air cooled bainitic structure is that the transformation has a natural tendency to reject hydrogen gas and the steel would be virtually free from hydrogen flaking unlike that in an alloy steel. The steel in the present case was manufactured by continuous casting while ingot casting is also possible. Macro segregation was minimised by having low carbon and sulphur contents. The steel can be hot or cold charged during deformation. The as-cast steel is amenable for hot deformation using hot forging and hot rolling and in this specific case it was directly hot rolled with a reduction ratio more than 4 with a cross section of round corner square.

The hot deformation temperature at which thermo-mechanical processing is carried out is between 1280 and 850 °C. The plastic deformation of the steel happens with good plastic flow behaviour and with no surface defects. The finish rolling temperature was maintained in a range between 1000 to 900°C. The steel after thermo-mechanical processing was subject to initially three different cooling rates using vermiculite cooling, air cooling or water quenching. Each of the three cooling methods leads to the formation of predominantly bainitic microstructure. The typical mechanical properties achieved in the 35 MT directly hot rolled steel are shown in Table 3. The corresponding microstructures are shown in Figure 2.

**Table 2: Properties of raw material achieved at three cooling conditions.**

| **Type of cooling** | **Direction** | **UTS (MPa)** | **YS (MPa)** | **%E** | **%RA** | **CVN (J)** | **Hardness HB** |
|---|---|---|---|---|---|---|---|
| Vermiculite Cooled | Longitudinal | 1140 | 767 | 14.8 | 45 | 12.41 | 332 |
| | Transverse | 1108 | 762 | 10.2 | 25 | 10.45 | |
| Air cooled | Longitudinal | 1137 | 761 | 17.8 | 46 | 17.6 | 340 |
| | Transverse | 1178 | 784 | 12 | 31 | 11.3 | |
| Water quenched | Longitudinal | 1195 | 861 | 16 | 30 | 20.58 | 352 |
| | Transverse | 1189 | 850 | 9.8 | 29 | 9.15 | |

This example shows that the steel is amenable for processing to bainitic transformation after thermo-mechanical processing over a wide range of temperatures. This implies that the steel exhibits bainitic structure with lesser control of cooling rate. This simplifies the manufacturing process in closed die forging where in some cases desired cooling rate is imposed to get a specific microstructure. The present invention confirms that there is no need for forced air cooling or a very controlled cooling in the conveyor after deformation. The steel made using the process of invention was used in making of close die steel component, where excellent consistency in mechanical properties is achieved.

The mechanical properties obtained in this study shows ultra-high strength range consistent in a product. Such levels of properties are usually achieved in hardened and tempered steels. In the case of the present invention, there is no need for hardening and tempering and air cooling is sufficient to achieve the desired mechanical properties. It was also observed that the transverse properties as shown in Table 2 significantly improved when the steel was subject to thermo-mechanical processing in a closed die forging operation.

The steel bar manufactured using the invented process, are easy to forge into complex shaped components. The forging made of such steel had the desired bainitic structure. This ultra-high strength steel contributes to weight reduction of the existing components that enhances fuel efficiency in automotive type applications. The component weight reduction can be achieved by at least 10%.

In an extended study, the steel made using the process of invention was used for forging an automotive front axle beam designed for Gross Axle Weight Rating (GAWR) of about 7 tons as shown in Figure 3. The closed die forging of components made using the steel of the invention can be manufactured using a hammer or a press, and the forging process involves soaking of rolled bar at a temperature range between 1280° C and 1220° C , The Finish forging temperature is maintained within temperature range 1000 to 900°C. The forging process involves preform manufacturing step for blocker forging and finisher forging, the process of preform manufacturing consist of reduce rolling the heated billet and bending some portion using bender tool. The finish forging is followed by cooling the hot forged component in any of the cooling medium selected from a group comprising controlled cooled, air, oil, or polymer. The microstructure of forging component using the ultra-high strength steel is as shown in Figure 4.

It should be noted that the steps of forging process disclosed in the example above are specific to the axle beam type components. Forging process for other types of components manufactured using the steel of the invention may vary depending on component geometry.

The mechanical properties and fatigue testing of the beam was carried out. The mechanical properties and the performance of the steel are as given in Table 3. The test results shown superior fatigue properties of steel of the present invention as compared to the conventional quench tempered medium carbon steel AISI 1045 and alloy steel DIN 40Cr4.

**Table 3: Typical mechanical property performance of the steel of the invention after forging into components.**

| **Type of cooling** | **YS (MPa)** | **UTS (MPa)** | **%E** | **%RA** | **Impact (J)** | **Hardness HB** |
|---|---|---|---|---|---|---|
| Air Cooled | 700-800 | 1100-1200 | 13-18 | 35-45 | 20J | 331-352 |
| Oil Quenched | 890-980 | 1300-1380 | 10-15 | 32-50 | 23J | 412-425 |
| Water Quenched | 980-1030 | 1350-1420 | 12-17 | 34-50 | 27J | 417-438 |

The fatigue test results shows at least five times better fatigue life as compared to conventional heat treated steel grades such as AISI 1045, 40Cr4. Axle beams made from the invention of the present steel can be made slimmer than those made with micro alloyed steel grades (30MnVS6+Ti) resulting in weight reduction.

### Benefits of the steel of the invention over other steel grades:

The steel shows dense sheaves of bainitic ferrite with nano-carbides. The strengths developed in this invention far surpass the traditional medium carbon microalloyed steel grades used for component fabrication.

One key feature of the process of the present invention is that the enhanced strength of the steel disclosed herein is achieved without heat treatment by cooling in air or cooling in other media after thermo-mechanical processing. The mechanical properties of the steel of the invention are comparable to that in the oil hardened and tempered alloy steels and superior to that obtained in ferrite pearlitic medium carbon microalloyed steel.

Unlike alloy steels which obtain ultra high strength levels after quenching and low temperature tempering, the present steel achieves the strength value merely using thermo-mechanical processes and with suitable cooling medium. The steel of the present invention is comparable with 1% Cr alloy steel in terms of cost but it has mechanical properties which are equivalent to alloy steels with further alloying additive and heat treatment. The enhanced strength enables reduction in weight of the components in range of at least 10 % in case of the traditional medium carbon micro alloyed steel. The improved strength values have resulted in improved fatigue life of components made from the steel of the present invention is at least 5 times when compared with those which were made using traditional micro alloyed steel grade. In the case of automotive components, the steel of the present invention is useful for light-weighting opportunities in applications such as shafts, axle beams, steering knuckles, connecting rods, camshaft, etc.

In summary, the present invention has the following aspects and advantages:
1. A robust chemistry of the steel was developed from as-cast ingot or concast product which can be hot forged or hot rolled followed by controlled cooling in media such as vermiculite cooling, air cooling, oil cooling or polymer show ferrite-carbidic bainitic microstructure that exhibits ultra high strength levels with good ductility and reasonable toughness.
2. The steel has a composition as specified in claim 1. The Oxygen is maintained at a level of less than 15 ppm to ensure cleanliness for the ultra-high strength range.
3. The steel which is thermo-mechanically processed and can be subject to a wide variety of cooling condition to give bainitic structure namely vermiculite cooling, air cooling, oil cooling, polymer quenching or water quenching exhibit bainitic structure and a wide variety of properties in the ultra high strength range with good ductility and reasonable toughness.
4. The steel could be manufactured in large tonnages and present study has resulted in a 35 MT electric arc furnace steel making furnace followed by continuous casting and it could be hot forged and hot rolled without defects at a temperature range between 850 and 1280°C. The steel developed was extensively studied for mechanical properties in as-rolled, as-forged and closed die forging condition followed by air cooling where excellent Ultra high strength- ductility properties could be achieved.
5. The components like front axle beam have been analysed for fatigue performance. The steel shows at least five times the fatigue life of the corresponding alloy steel component. Thus, the steel developed has a potential opportunity to replace expensive alloy steels processed by quenching and tempering treatment and produce lightweight component with better strength to weight ratio. Weight reduction of structural component of at least 10 % can be achieved.

## Claims

1. An ultra-high strength steel of present invention **characterised in that** the said steel comprises in weight percentage:
carbon in the proportion of 0.1 to 0.25%,
manganese in the proportion of 1.2 to 2.5%,
silicon in the proportion of 0.5 to 1.7 %,
chromium in the proportion of 0.8 to 1.4 %,
molybdenum in the proportion of 0.05 to 0.1%,
niobium in the proportion of 0.05 to 0.10%,
titanium in the proportion of 0.01 to 0.035%,
and the residual elements less than 0.4%, wherein the residual elements are:
nickel in the proportion of less than 0.4%,
vanadium in the proportion of less than 0.1%,
sulphur in the proportion of less than 0.03%,
phosphorus in the proportion of less than 0.02%,
wherein the steel further comprises in weight percentage:
aluminium in the proportion of less than 0.02%,
boron less than 30 ppm,
oxygen in an amount of less than 15 ppm,
and balance iron and any unavoidable impurities.

2. A process of making an ultra-high strength steel rolled bar, the said process comprising the steps of:
- melting the steel of the chemical composition disclosed in claim 1, followed by secondary refining and vacuum degassing, wherein said secondary refining comprises the step of killing with aluminium to bring the oxygen level in said steel to under 15 ppm,
- casting of said steel through ingot casting or continuous casting into a bloom,
- hot charging the as-cast ingot or the continuously cast bloom, or alternatively, cold-charging them in a furnace,
- soaking said ingot or said bloom at a temperature range between 1280 °C and 1220 °C,
- subjecting said soaked bloom to hot rolling,
- carrying out reduce rolling,
- finish rolling at a temperature range 1000 to 900°C,
- control cooling the hot rolled steel in any of the cooling medium selected from a group comprising vermiculite, air, oil, polymer, or water.

3. A process of making forged components with an ultra-high strength steel, **characterised in that** said process comprises the steps of:
- heating and soaking of rolled bar made using the process disclosed in claim 2 at a temperature range between 1280 °C and 1220 °C,
- hot forging of component,
- finish forging the component at a temperature range 1000 to 900°C,
- cooling the finish forged component in any of the cooling medium selected from a group comprising controlled cooled, air, oil, or polymer.

4. A process of making an ultra-high strength steel as claimed in claims 1 and 2, **characterised in that** melting in the step of casting is carried out using an induction furnace or an electric arc furnace or a basic oxygen furnace.

5. A process of making an ultra-high strength steel as claimed claim 4, **characterised in that** the step of thermo-mechanical processing is carried out by a technique selected from a group comprising hot rolling, or closed die forging, or extrusion.

6. A process of making forged components as claimed in claim 3, **characterised in that** the step of hot forging of component comprises the step of preform manufacturing for blocker forging and finisher forging, followed by cooling.

7. A process of making forged components as claimed in claim 6, **characterised in that** the step of preform manufacturing comprises the steps of reduce rolling and bending.

## Patentansprüche

1. Ultrahochfester Stahl der vorliegenden Erfindung, **dadurch gekennzeichnet, dass** der Stahl in Gewichtsprozent umfasst:
Kohlenstoff im Anteil von 0,1 bis 0,25%,
Mangan im Anteil von 1,2 bis 2,5%,
Silizium im Anteil von 0,5 bis 1,7 %,
Chrom im Anteil von 0,8 bis 1,4 %,
Molybdän im Anteil von 0,05 bis 0,1%,
Niob im Anteil von 0,05 bis 0,10%,
Titan im Anteil von 0,01 bis 0,035%,
und dass die restlichen Elemente weniger als 0,4% betragen, wobei die restlichen Elemente sind:
Nickel im Anteil von weniger als 0,4 %,
Vanadium im Anteil von weniger als 0, 1%,
Schwefel im Anteil von weniger als 0,03%,
Phosphor im Anteil von weniger als 0,02%,
wobei der Stahl weiterhin in Gewichtsprozent umfasst:
Aluminium im Anteil von weniger als 0,02%,
Bor weniger als 30 ppm,
Sauerstoff in einer Menge von weniger als 15 ppm,
Rest Eisen und unvermeidbare Verunreinigungen.

2. Verfahren zur Herstellung eines Walzstabs aus ultrahochfestem Stahl, wobei das Verfahren die folgenden Schritte umfasst:
- Schmelzen des Stahls mit der in Anspruch 1 offenbarten chemischen Zusammensetzung, gefolgt von sekundärer Raffination und Vakuumentgasung, wobei die sekundäre Raffination den Schritt des Tötens mit Aluminium umfasst, um den Sauerstoffgehalt in dem Stahl auf unter 15 ppm zu bringen,
- Gießen des Stahls durch Blockguss oder Strangguss zu einem Vorblock,
- Heißchargieren des Gussblocks oder des Stranggussblocks oder alternativ Kaltchargieren derselben in einem Ofen,
- Tauchen des Barrens oder des Vorblocks in einem Temperaturbereich zwischen 1280 °C und 1220 °C,
- Warmwalzen des getauchten Vorblocks,-
- Durchführung von Reduzierwalzen,
- Fertigwalzen in einem Temperaturbereich von 1000 bis 900 °C,
- geregeltes Kühlen des warmgewalzten Stahls in einem beliebigen Kühlmedium, das aus einer Gruppe ausgewählt wird, die Vermiculit, Luft, Öl, Polymer oder Wasser umfasst.

3. Verfahren zur Herstellung geschmiedeter Bauteile mit einem ultrahochfesten Stahl, **dadurch gekennzeichnet, dass** das Verfahren die folgenden Schritte umfasst:
- Erhitzen und Tauchen von nach dem in Anspruch 2 offenbarten Verfahren hergestellten Walzstäben in einem Temperaturbereich zwischen 1280 °C und 1220 °C,
- Warmschmieden des Bauteils,
- Fertigschmieden des Bauteils in einem Temperaturbereich von 1000 bis 900 °C,
- Kühlen des fertig geschmiedeten Bauteils in einem beliebigen Kühlmedium, das aus einer Gruppe ausgewählt wird, die geregelt gekühlte Luft, Öl oder Polymer umfasst.

4. Verfahren zur Herstellung eines ultrahochfesten Stahls nach Anspruch 1 und 2, **dadurch gekennzeichnet, dass** das Schmelzen im Schritt des Gießens unter Verwendung eines Induktionsofens oder eines elektrischen Lichtbogenofens oder eines Linz-Donawitz-Ofens durchgeführt wird.

5. Verfahren zur Herstellung eines ultrahochfesten Stahls nach Anspruch 4, **dadurch gekennzeichnet, dass** der Schritt der thermo-mechanischen Verarbeitung durch eine Technik durchgeführt wird, die aus einer Gruppe ausgewählt wird, die Warmwalzen, Gesenkschmieden oder Strangpressen umfasst.

6. Verfahren zur Herstellung geschmiedeter Bauteile nach Anspruch 3, **dadurch gekennzeichnet, dass** der Schritt des Warmschmiedens eines Bauteils den Schritt der Herstellung einer Vorform für das Blockschmieden und das Fertigschmieden umfasst, gefolgt von Abkühlen.

7. Verfahren zur Herstellung geschmiedeter Bauteile nach Anspruch 6, **dadurch gekennzeichnet, dass** der Schritt des Herstellens der Vorform die Schritte des Reduzierwalzens und Biegens umfasst.

## Revendications

1. Acier à ultra-haute résistance selon la présente invention, **caractérisé en ce que** ledit acier comprend en pourcentage en poids :
du carbone dans la proportion de 0,1 à 0,25 %,
du manganèse dans la proportion de 1,2 à 2,5 %,
du silicium dans la proportion de 0,5 à 1,7 %,
du chrome dans la proportion 0,8 à 1,4 %,
du molybdène dans la proportion de 0,05 à 0,1 %,
du niobium dans la proportion de 0,05 à 0,10 %,
du titane dans la proportion de 0,01 à 0,035 %,
et les éléments résiduels à raison de moins de 0,4 %, dans lequel les éléments résiduels sont :
du nickel dans la proportion inférieure à 0,4 %,
du vanadium dans la proportion inférieure à 0,1 %,
du soufre dans la proportion inférieure à 0,03 %,
du phosphore dans la proportion inférieure à 0,02 %,
dans lequel l'acier comprend en outre en pourcentage en poids :
de l'aluminium dans la proportion inférieure à 0,02 %,
du bore à raison de moins de 30 ppm,
de l'oxygène en une quantité inférieure à 15 ppm,
et le reste étant constitué de fer et de quelconques impuretés inévitables.

2. Procédé de fabrication d'une barre laminée en acier à ultra-haute résistance, ledit procédé comprenant les étapes consistant à :
- faire fondre de l'acier de la composition chimique décrite dans la revendication 1, puis procéder à un affinage secondaire et à un dégazage sous vide, dans lequel ledit affinage secondaire comprend l'étape de destruction par de l'aluminium pour amener le taux d'oxygène dans ledit acier à moins de 15 ppm,
- couler ledit acier par coulée en lingot ou coulée continue en un bloom,
- charger à chaud le lingot de coulée ou le bloom coulé en continu, ou en variante, les charger à froid dans un four.
- tremper ledit lingot ou ledit bloom à une température comprise entre 1 280°C et 1 220°C,
- soumettre ledit bloom trempé à un laminage à chaud,
- réaliser un laminage de réduction,
- terminer le laminage à une température de 1 000 à 900°C,
- contrôler le refroidissement de l'acier laminé à chaud dans l'un quelconque milieu de refroidissement choisi dans un groupe comprenant de la vermiculite, de l'air, de l'huile, un polymère ou de l'eau.

3. Procédé de fabrication de composants forgés avec un acier à ultra-haute résistance, **caractérisé en ce que** ledit procédé comprend les étapes consistant à :
- chauffer et tremper une barre laminée réalisée en utilisant le procédé décrit dans la revendication 2 dans une température comprise entre 1 280°C et 1 220°C,
- forger le composant à chaud,
- terminer le forgeage du composant dans une plage de température de 1 000 à 900°C,
- refroidir le composant forgé de finition dans l'un quelconque moyen de refroidissement choisi dans un groupe comprenant de l'air, de l'huile ou un polymère refroidi(e) de manière régulée.

4. Procédé de fabrication d'un acier à ultra-haute résistance selon les revendications 1 et 2, **caractérisé en ce que** la fusion lors de l'étape de coulée est effectuée à l'aide d'un four à induction ou d'un four à arc électrique ou d'un four à oxygène basique.

5. Procédé de fabrication d'un acier à ultra-haute résistance selon la revendication 4, **caractérisé en ce que** l'étape de traitement thermomécanique est réalisée par une technique choisie dans un groupe comprenant le laminage à chaud, ou le forgeage à matrice fermée, ou l'extrusion.

6. Procédé de fabrication de composants forgés selon la revendication 3, **caractérisé en ce que** l'étape de forgeage à chaud du composant comprend l'étape de fabrication de préforme pour un forgeage de blocage et un forgeage de finition, suivie d'un refroidissement.

7. Procédé de fabrication de composants forgés selon la revendication 6, **caractérisé en ce que** l'étape de fabrication de préforme comprend les étapes de laminage de réduction et de flexion.
